

Oct. 14, 1941.

J. R. HILL

2,258,609

NONHALATION PHOTOGRAPHIC ELEMENT

Filed Sept. 26, 1938



INVENTOR.  
John R. Hill.

BY

*Lynn B. Morris*

ATTORNEY

## UNITED STATES PATENT OFFICE

2,258,609

## NONHALATION PHOTOGRAPHIC ELEMENT

John R. Hill, Parlin, N. J., assignor to Du Pont  
Film Manufacturing Corporation, New York,  
N. Y., a corporation of Delaware

Application September 26, 1938, Serial No. 231,818

6 Claims. (Cl. 95—9)

This invention relates to a light-sensitive photographic element having a removable backing; more particularly, it relates to a light sensitive photographic film having a removable light absorbing backing; still more particularly it relates to a light-sensitive photographic film having a water-insoluble removable backing containing a dye which is absorptive of light of all wave lengths to which the film is sensitive.

It is an object of this invention to provide a water-insoluble coating for light sensitive photographic elements which may readily be removed from the same by organic solvents. A further object is to provide a removable backing for a photographic film containing a solvent soluble dye in which the dye will not transfer to the base during storage. A still further object is to provide a removable dyed anti-halation coating for photographic film elements which are free from tackiness and photographic active substances and have a resistance to abrasive forces when dry. Still other objects will be apparent from a consideration of the hereinafter described invention.

The above and other objects are accomplished by the use of water-insoluble organic solvent-soluble lower alkyl ethers of cellulose. In a more limited sense the invention comprises a photographic element having a sensitized emulsion upon one side of a transparent support and a coating of a cellulose lower alkyl ether of the type which is insoluble in water and is not injuriously softened thereby, but which is soluble in water-soluble monohydric alcohols and water-alcohol mixtures and contains dye which is absorptive of light of all wave lengths to which said emulsion is sensitive. The dyes may vary widely in chemical structure and properties but should be soluble to the extent of at least 1% in an organic solvent.

In the preferred embodiment of the invention, the removable backing coating is composed of methyl cellulose or ethyl cellulose which is insoluble in water and is not injuriously affected thereby, but is soluble in ethanol or a water-ethanol mixture containing at least 50% and preferably at least 70% of the latter, and a dye having the above-described absorption characteristics.

The cellulose ethers in general should have an alkoxy content of at least 2.2 mols per C<sub>6</sub> unit of the cellulose nucleus. In the case of ethyl cellulose it has been found that an ethoxy content of 2.43 to 2.54 mols per C<sub>6</sub> unit and a viscosity of 45 to 50 centipoises (determined on a 5%

solution in a mixture of 80% toluene and 20% ethanol by volume at 25° C.) gives an excellent product for use according to this invention which has a maximum solubility in ethanol and other solvents. The ethyl ethers of cellulose having the above-described characteristics are preferred.

In investigating these ethers the surprising discovery was made that the addition of a dye to the cellulose ether before coating of the same upon the base had a very definite effect upon the adherence of the same to the film base. For instance, it was found that when ethyl cellulose was coated upon a cellulose acetate film base the dry layer could be stripped off even though the coating solution contained an active solvent for the base. Upon adding a dye to the coating it became more adherent. The adherence was found to be more pronounced if the ratio of the dye was controlled within the narrow limits of 0.5 to 0.9 part of dye to one part of cellulose ether.

The invention will be further illustrated but is not intended to be limited by the following examples in which the parts stated are parts by weight unless otherwise indicated.

In the accompanying drawing a film support 1 composed of a transparent cellulose derivative has coated on its upper surface a light sensitive silver halide emulsion 2 and on its rear surface 30 an anti-halation coating 3 composed of a water-insoluble alcohol-soluble cellulose lower alkyl ether and an anti-halation material.

*Example I*

An alcohol soluble ethyl cellulose having a viscosity of 45 centipoises and an ethoxy content of 2.50 mols per C<sub>6</sub> unit was incorporated in the following composition:

|                       | Per cent |
|-----------------------|----------|
| Ethyl cellulose       | 1.5      |
| Nigrosine (C. I. 864) | 1.25     |
| Ethanol               | 97.25    |
|                       | 100.     |

45 which was coated by means of a beading roller on the back side of a transparent cellulose acetate film base which carried upon its face a panchromatic emulsion and allowed to dry. The coating was strongly adherent. The film was exposed in a camera, processed, and then placed into a bath containing 70% ethanol and 30% water, whereupon the backing layer was dissolved off. Upon examination the film was found to be entirely free from the backing coating and un-stained.

Similar results were obtained by substituting equivalent amounts of the following spirit soluble dyes; Naphthol Blue-Black (C. I. 246), Durol Black (C. I. 307), Sulfon Blue (C. I. 208), Victoria Green (C. I. 657), Helvetia Green (C. I. 660), Brilliant Green (C. I. 662), Acid Green (C. I. 666), Wool Fast Blue (C. I. 833), Victoria Blue (C. I. 729), and Fast Black (C. I. 919) in similar amounts.

*Example II*

A coating solution of the following composition:

|                     | Per cent     |
|---------------------|--------------|
| Ethyl cellulose     | 1.5          |
| Magenta (C. I. 677) | 0.8          |
| Ethanol             | 97.7         |
|                     | <b>100.0</b> |

was coated upon the back of a film which carried upon its face an orthochromatic emulsion and dried. The coating was strongly adherent and free from coating streaks and tackiness. After exposure and processing the film was incorporated into a water-ethanol bath containing about 75% of the latter, whereupon the dyed backing layer was readily removed. Upon inspection the base was found to be clean and entirely free from stain and coating particles. The ethyl cellulose used in this example was water insoluble and had an ethoxy content of 2.48 mols per glucose unit.

Similar results were obtained when the specific dye of this example was substituted by equivalent amounts of Methyl Violet (C. I. 680), Crystal Violet (C. I. 681), Safranine (C. I. 841), Rhodamine (C. I. 749) and Ponceau 6R (C. I. 186).

*Example III*

A coating solution of the following composition:

|                         | Per cent |
|-------------------------|----------|
| Propyl cellulose        | 1.5      |
| Durol Black (C. I. 307) | 0.5      |
| Ethanol                 | 98.0     |

was coated upon the back of a film base which carried upon its face a panchromatic emulsion and dried. The coating was quite adherent, free from coating streaks and non-tacky. After exposure in a camera and processing the film was incorporated into a water-alcohol bath containing about 80% of the latter, whereupon the anti-halation layer was readily removed. After removal from the bath the base was found to be clean and entirely free from stain and coating particles. The propyl cellulose in this example contained a propoxy content of 2.48 mols per C<sub>6</sub> unit and was water insoluble.

In place of the specific ethers of the above examples any ether having the characteristics hereinbefore mentioned may be substituted. Thus, the cellulose isopropyl, butyl and isobutyl ethers which are alcohol or alcohol-water soluble, but water-insoluble may be substituted in like amount.

While it has been stated that the cellulose ether dyed layer is not soluble or removable in water alone, it is to be understood that this is to mean that it is so little affected during the period of time which it is in contact in aqueous solutions during the usual photographic processes that no visible change is apparent.

The ethers of this invention are not only soluble in water-alcohol mixtures and water soluble alcohols, but are soluble in organic solvents in general. Thus, it is not necessary to use only water-

alcohol removal solutions. Other organic solvents may be mixed with the alcohols or water-alcohol mixtures or the former may be used alone. It is to be understood, however, that the water-alcohol mixtures are the preferred removal solvents. As examples of other solvents mention is made of ethyl ether, chlorinated hydrocarbons, e. g. chloroform, carbon tetrachloride, trichloroethylene; acetone, methyl alcohol, benzene, toluene, xylene, nitrobenzene, etc. and mixtures thereof. The solvents used, however, should not affect the film base. As examples of other useful water-soluble alcohols, mention is made of methanol, isopropanol, n-propanol and n-butanol. These may be used in admixture with the above solvents.

In general, any dye which possesses the property of absorbing actinic light, of being readily dissolved or destroyed in ordinary photographic baths and of not injuring such baths may be used. The dye or dyes to be used in any specific instance are primarily determined by the light sensitivity of the emulsion. Such emulsions are usually gelatin silver halide emulsions which contain sensitizers such as cyanine, carbocyanine, psuedo-cyanine, cyazine bases and salts. That is, it must be absorptive of light of the wave lengths to which the emulsion is sensitive. In general the dye should be added in an amount sufficient to give a photographic density of 0.8 or the amount of dyed layer should be sufficient to give such a density. As examples of additional useful dyes, mention is made of:

|                                                      |
|------------------------------------------------------|
| Auramine (C. I. 655)                                 |
| Helianthin (C. I. 142, 146)                          |
| Brilliant Yellow S (C. I. 144)                       |
| Chrysoin (C. I. 148)                                 |
| Acid Blue Black (C. I. 246)                          |
| Rhodamine (C. I. 749, 750, 751, 746, 753, 761, 763)  |
| Fuchsin (C. I. 677)                                  |
| Safranine G (C. I. 841)                              |
| Ponceau 6R (186)                                     |
| Crocein Scarlet (C. I. 277, 251, 286, 252, 291, 183) |
| Azorubin (C. I. 179)                                 |
| Safranine O (C. I. 841)                              |
| Ponceau 2R (C. I. 79)                                |
| Spirit Solution Nigrosine (C. I. 864)                |
| Metanil Yellow (C. I. 138)                           |

This invention possesses the advantage that a nontacky anti-halation layer which is readily soluble in alcohol and water alcohol mixtures may be quickly prepared. A further advantage resides in the fact that a non-halation layer which is strongly adherent to film base may be economically prepared. A still further advantage is that a film which is not stained by a dyed anti-halation layer is provided. Other advantages will be apparent to those skilled in the art.

As many apparently widely different embodiments of this invention may be made without departing from the spirit and scope thereof, it is to be understood that I do not limit myself to the specific embodiments herein except as defined by the appended claims.

I claim:

1. A photographic film element comprising a light-transmitting support, a light sensitive emulsion layer on one face thereof and a layer consisting of a water-insoluble ethyl cellulose which is soluble in water-ethanol mixtures predominating in the latter, said layer containing from 0.5 to 0.9% of a dye which is absorptive of light of all wave lengths to which said emulsion is sensitive carried upon the opposite face.

2. A photographic element comprising a light transmitting support, a light sensitive emulsion layer on one face thereof and a layer consisting of a water-insoluble ethyl cellulose which is soluble in ethanol-water mixtures containing at least 70% of the former, said layer containing from 0.5 to 0.9% of a dye which is absorptive of all wave lengths to which said emulsion is sensitive carried upon the opposite face.

3. A photographic element comprising a light transmitting support, a light sensitive emulsion layer on one face thereof and a layer consisting of a cellulose ethyl ether having an ethoxy content of 2.43 to 2.54 mols per C<sub>6</sub> unit, said layer containing from 0.5 to 0.9% of a material which absorbs actinic light carried upon the opposite face.

4. A photographic element comprising a light transmitting support, a light sensitive silver halide emulsion layer on one face thereof and a layer consisting of a cellulose ethyl ether having an ethoxy content of 2.43 to 2.54 mols per C<sub>6</sub> unit, said layer containing from 0.5 to 0.9% of a dye

which is absorptive of light of all wave lengths to which said emulsion is sensitive carried upon the opposite face.

5. A photographic film element comprising a light transmitting support, a light sensitive emulsion layer on one face thereof and a layer consisting of a water-insoluble cellulose lower alkyl ether which is soluble in water-ethanol mixtures predominating in the latter, said layer containing from 0.5 to 0.9% of a dye which is absorptive of light of wave lengths to which said emulsion is sensitive.

6. A photographic film element comprising a light transmitting support, a light sensitive silver halide emulsion layer on one face thereof and a layer consisting of a water-insoluble cellulose lower alkyl ether which is soluble in water-ethanol mixtures predominating in the latter, said layer containing from 0.5 to 0.9% of a dye which is absorptive of light of wave lengths to which said emulsion is sensitive.

JOHN R. HILL.